

March 19, 1968

**1968 H. J. H. VAN DEUTEKOM 3,3**  
METHOD OF COATING A MAGNETOSTRICTIVE MATRIX PANEL  
WITH A DAMPING MASS AND RESULTING ARTICLE  
Filed July 6, 1964

3,374,109

Filed July 6, 1964



**FIG.1**



**FIG.2**

INVENTOR.

## HUIBERT JACOBUS HENDRIK VAN DEUTEKOM

BY

Frank R. Sifari  
AGENT

AGENT

3,374,109

## METHOD OF COATING A MAGNETOSTRICTIVE MATRIX PANEL WITH A DAMPING MASS AND RESULTING ARTICLE

Huibert Jacobus Hendrik van Deutekom, Emmasingel, Eindhoven, Netherlands, assignor to North American Philips Company, Inc., New York, N.Y., a corporation of Delaware

Filed July 6, 1964, Ser. No. 380,341

Claims priority, application Netherlands, July 12, 1963, 295,257

3 Claims. (Cl. 117—201)

### ABSTRACT OF THE DISCLOSURE

The magnetostrictive vibrations in a magnetic core storage matrix panel are damped by coating matrix with a mixture of a high-molecular weight polyvinylbutyral resin and a plasticizer such as tricresylphosphate.

The invention relates to the production of a damped matrix by coating it with a damping mass suitable for damping mechanical vibrations at temperatures lying between about  $-10^{\circ}$  C. and about  $+80^{\circ}$  C., which vibrations may occur, for example, in magnetic core storages as a result of the electric pulses applied to the storage.

A magnetic core storage usually comprises at least one matrix panels, each of which is formed by a number of toroidal cores arranged in rows and columns through which insulated electric conductors are threaded. A matrix panel may furthermore comprise so-called blocking wires and a read wire, which are threaded through the cores in a given, known pattern.

The cores are formed by rings usually consisting of an oxidic magnetic material having a substantially rectangular hysteresis loop.

When magnet cores are employed as storage elements, it is desirable that mechanical vibrations which may be performed by the cores under the action of the applied electric pulses owing to their magneto-strictive properties should be restricted as far as possible without adversely affecting the magnetic properties of the elements. The magneto-strictive properties of the storage elements may result in that with certain patterns of information stored in the storage, the so-called worst pattern, reading may give erroneous information. Besides, any motion performed by the cores with respect to the electric conductors under the action of vibrations from without may give rise to wear and breakage of the electric conductors.

The invention has for its object to produce matrix coated with a damping mass which has a negligible influence on the electro magnetic properties of the cores, which damps the magneto-strictive vibrations, which raises the resonance frequency of the matrix panel and the properties of which will not vary with time.

In accordance with the invention such a mass is obtained by making a mixture of a plasticizer and high-molecular polyvinylbutyral resin in a ratio by weight from 1:1 to 3:7 and a volatile, organic solvent in a quantity such that a workable mass is obtained.

Best results are obtained by using a polyvinylbutyral resin having a *k*-value of its intrinsic or own viscosity of at least 50.

A plasticizer providing by mixing with a polyvinylbutyral resin a damping mass of practical suitability must satisfy the following requirements:

(1) The softener must be miscible in adequate quantities with polyvinylbutyral resin and must remain miscible in such quantities in a wide temperature range.

(2) The vapour pressure of the softener must be low in the desired temperature range.

(3) In the desired temperature range the viscosity of the mixture of this softener with the polyvinylbutyral resin must be substantially constant.

(4) The mixture must be self-extinguishing.

(5) The mixture must be removable for carrying out repairs.

(6) The mixture must be little aggressive or not at all.

10 It has been found that tricresylphosphate fulfils all these requirements in a particularly satisfying manner.

A mass according to the invention may be produced in the following manner.

15 100 gms. of tricresylphosphate is dissolved in 1000 mls. of ethanol; then 100 gms. of polyvinylbutyral resin is gradually added, whilst stirring, to the solution until the mixture is clear. A quantity of an organic colouring substance may be added to the mixture, in order to facilitate the application of the mass. Satisfactory results are obtained by using a polyvinylbutyral resin which has a *k*-value of its own viscosity of 50 to 55 (Fikentscher: Cellulose Chemie 13, pages 58 and ff., 1932). This mass is preferably employed when the widest possible temperature range has to be covered, whilst very small cores are used.

20 25 It may be used at temperatures lying between  $-10^{\circ}$  C. and  $+40^{\circ}$  C. and for a short time up to  $+80^{\circ}$  C. At  $+100^{\circ}$  C. dripping effects do not yet occur. The mixture is self-quenching and does not maintain combustion even at very high temperatures. If the requirements are less

30 severe or if cores of not too small dimensions are used, a smaller quantity of tricresylphosphate or of other plasticizer may suffice. In general, however, the quantity to be used will not be less than 30% of the total weight of the mixture of plasticizer and the polyvinylbutyral resin.

35 Use is preferably made of a rapidly evaporating, non-aggressive or little aggressive solvent, for example methanol, ethanol and the like. The mass is applied to the matrix panel by casting, painting, dipping or the like. Then the solvent is evaporated for example by heating at about

40  $+70^{\circ}$  C.

Other plasticizers which can be used include tricrelenylphosphate, cresyldiphenyl phosphate and tri-(2 ethyl phenyl) phosphate.

45 The effect of the damping mass will be explained more fully with reference to the accompanying drawing and to measurements to be described hereinafter.

In the drawing FIG. 1 shows diagrammatically part of a matrix panel.

50 FIG. 2 shows an idealised hysteresis loop.

Referring to FIG. 1 reference numeral 19 designates the cores of oxidic ferromagnetic material X and Y designate the electric conductors used for recording and reading the information. The arrows indicated near the conductors indicate for each conductor the direction in which the pulse has to be passed through the wire for writing information, Z is the blocking wire through which a pulse can be guided for reading in order not to loose information during reading and writing, so it is avoided that additional information is written, when a plurality of matrix panels co-operate. S is the read wire. During reading pulses are introduced in said wire, from which pulses the information available in the matrix panel can be inferred. Owing to the manner of twisting of the wires disturbing pulses neutralise each other for the major part.

60 65 With this manner of twisting the cores are divided into two groups of equal size, which supply pulses of opposite polarities, both when the magnetization in cores changes over and when the magnetization varies under the action of pulses which are not sufficiently great for producing the change-over of the magnetisation. When pulses are passed through the read wire S, the value of which suffers for

changing over the magnetisation of the cores, a pattern of information is written in the matrix panel, which is known under the name of "worst pattern." With such a pattern all cores inducing a positive pulse in the read wire at the changeover of the magnetisation are in a state of positive remanence and all cores inducing a negative pulse under the same conditions are in a state of negative remanence or conversely in accordance with the polarity of the pulses passed through the read wire, when this pattern is induced.

It is found that with such a pattern the neutralisation of disturbing pulses is at a maximum, whilst the residual signal due to the incomplete neutralisation is at the maximum.

With such a pattern the effect of a damping mass on the magnetostrictive vibrations can be measured particularly satisfactorily from the disappearance of the vibration of the disturbing pulses on the read wire.

FIG. 2 shows the ideal hysteresis loop of a core associated with a given current strength  $I_m$  corresponding to a field strength  $H_m$ .  $B^+m$  is the maximum induction.  $B^+r$  is the positive remanent induction.  $B^-r$  is the negative remanent and  $B^-m$  is the minimum induction. If the magnetic core is in the state of positive remanence 1 ( $B^+r$ ), a pulse  $-I_m$  corresponding to a field  $-H_m$  will cause the path 1-7-2-17-3 to be followed. When the field is removed, the magnetic core arrives in the state of negative remanence indicated as point 4 ( $B^-r$ ). When a pulse  $+I_m$  is passed through the conductors which corresponds to a field  $+H_m$ , the path 4-5-18-6 is followed and after the removal of the field the core returns to the state of positive remanence. When a pulse  $-1/2 I_m$  is passed through one of the conductors of the core, corresponding to a field  $-1/2 H_m$  (for example in recording information in the matrix panel in a number of cores), for example the point M is reached. When the field  $-1/2 H_m$  is removed, the core arrives at the state of remanent induction 8, which is, however, lower than the initial remanent induction  $B^+r$ . This process usually appears several times in a matrix panel. The permanent magnetic induction may then approach a limit value  $B^{+rd}$ . When a pulse  $-I_m$  corresponding to a field  $-H_m$  is passed through the conductors of the core, a flux variation occurs, which is proportional to the induction variation  $B^-m - B^{+rd}$ . Thus the read wire has produced across it a voltage pulse, the maximum value of which is indicated by  $rV1$  (read disturbed one). The usability of a damping mass has to fulfill the requirement that the maximum value of the voltage pulse across the read wires  $rV1$ , designated hereinafter by the  $rV1$ -signal, should not vary. A variation of the value of the signal would mean that the magnetic properties of the cores vary by the use of the damping mass.

In order to assess the favourable effect of the use of a damping mass prepared by the method according to the invention the following measurements were carried out:

(A) A matrix panel comprising 64 x 64 toroidal cores 19 having an outer diameter of 1.27 mm. and an inner diameter of 0.76 mm. of oxidic, ferromagnetic material, the hysteresis loop approaches the rectangular shape, and provided with a wiring as shown in FIG. 1 was covered by a mass consisting of a mixture of equal parts by weight of tricresylphosphate and high-molecular polyvinylbutyral resin having a  $k$ -value of the natural viscosity between 50 and 55, as indicated above.

The resonance frequency of the matrix panel was prior to lacquering 44 c./s.

After lacquering it was 59 c./s.

Two days after lacquering it was 72 c./s.

The resonance frequency was measured with the aid of a vibration table and a stroboscope.

(B) Prior to and after the application of the damping mass to the matrix panel the so-called  $rV1$  signal was mea-

ured. The measurements were carried out at 0° C. Any influence of the damping mass on the magnetic properties of the cores is at this temperature greater than at room temperature at a higher temperature.  $I_m$  was at this temperature 596 ma.

It was found that the value of the  $rV1$  signal prior to and after the application of the damping mass and after ageing of the damping mass was substantially the same. It may be concluded therefrom that the influence of the damping mass on the magnetic properties of the cores is only very slight.

When silicon lacquers are used, said influence appeared to be so high, particularly after ageing—the  $rV1$  signal decreased by at least about 20%—that this material is, in general, less suitable or not suitable at all.

(C) Prior to and after the application of the damping mass the residual signal due to the incomplete relative neutralisation of the disturbance pulses resulting from magnetostrictive vibrations of the cores was measured. It has been found in this respect that the noise of the read signal produced by pulses across the blocking wire has a magnetostrictive character. With a view to the magnetic-mechanical character of the vibration, it was found to be possible to damp mechanically these vibrations with the aid of the damping mass according to the invention. The measurements were carried out at +50° C., since it has in general been found that the damping effect of a damping mass decreases with an increasing temperature. The value of the pulse  $I_m$  was, at +50° C. 470 ma. The measurements were carried out on a matrix panel of the kind described under A; it comprised a "worst pattern" of information. The read signal was measured whilst a sequence of identical pulses was passed through the blocking wire; each had a value of 259 ma. (amplitude 60% of the amplitude of  $I_m$ ). The ratio between the voltage at the third vibration on the read wire due to the trailing edge of the pulse across the blocking wire was measured on a lacquered matrix panel and on a non-lacquered matrix panel. It was 1.5:13. The damping time, i.e. the time elapsing until the amplitude of the vibration is  $1/2$  of the maximum amplitude, was 24  $\mu$ sec. with a non-lacquered matrix panel and 3  $\mu$ sec. with a lacquered matrix panel. The frequency of the magnetostrictive vibrations was in both cases the same. Advantages of such a mass are furthermore, that it can be simply removed, for example by means of solvent, locally or wholly without damaging the matrix, for example for carrying out repairs and that it is self-extinguishing.

What is claimed is:

1. A method of producing a damped matrix by coating the matrix with a damping mass suitable for damping vibrations which may be produced in matrix panels, said damping mass comprising a mixture of a plasticizer and a high-molecular polyvinylbutyral resin in a ratio by weight of 1:1, to 3:7 and a volatile organic solvent in a quantity such that a workable mass is obtained.

2. A method as claimed in claim 1, characterized in that the matrix is coated with a mixture of tricresylphosphate and polyvinylbutyral resin having a  $k$  value of its own viscosity of 50 to 55.

3. Damped matrix panels obtained by the method of claim 1.

#### References Cited

#### UNITED STATES PATENTS

3,237,173 1/1962 Chamberlain et al. \_\_\_ 340—174

#### OTHER REFERENCES

"Polyisobutylene" Guterbock Springer, Verlag/Berlin 1959 (p. 178 relied on).

WILLIAM L. JARVIS, Primary Examiner.

UNITED STATES PATENT OFFICE  
CERTIFICATE OF CORRECTION

Patent No. 3,374,109

March 19, 1968

Huibert Jacobus Hendrik van Deutekom

It is certified that error appears in the above identified patent and that said Letters Patent are hereby corrected as shown below:

Column 2, line 71, "suffers" should read -- suffices --.

Signed and sealed this 2nd day of December 1969.

(SEAL)

Attest:

Edward M. Fletcher, Jr.

Attesting Officer

WILLIAM E. SCHUYLER, JR.

Commissioner of Patents